

## UNITED STATES PATENT OFFICE

LOUIS SCHULTE, OF PITTSBURGH, PENNSYLVANIA, ASSIGNOR TO ALLEGHENY STEEL COMPANY, OF BRACKENRIDGE, PENNSYLVANIA, A CORPORATION OF PENNSYLVANIA

## TIN-COATED CHROMIUM IRON ALLOY AND METHOD OF MAKING THE SAME

No Drawing.

Application filed May 25, 1926. Serial No. 111,626.

This invention relates to the electrodeposition of a sanitary metal, such as tin, on articles made from ferrous iron chromium alloys of the type of rustless iron, stainless steel and the like which contain chromium in the proportions of about 10% or 12%.

While such alloys are to a large extent stainless and rustless when hardened, tempered and polished, they have a less degree 10 of stainlessness or rustlessness when not hardened, tempered and polished.

There is a large and growing demand for stainless and rustless polished and mat surfaced sheets made from alloys of this type 15 for use in the manufacture of articles requiring deep stamping operations, but for such operations, the Brinell hardness should be under 350 and alloys of this type having a Brinell hardness under 350 do not have 20 the requisite degree of stainlessness and rustlessness.

An object of this invention is to produce articles such as sheets which are especially suitable for deep stamping operations, for 25 drawing and other working and which are stainless and rustless to a high degree.

A further object of this invention is to provide a method of surfacing alloys of this type in a way such as to materially increase 30 the stainlessness and rustlessness of articles made therefrom to an even higher degree than possessed by this type of alloy when hardened, tempered and polished and as heretofore furnished.

These, as well as other objects, which will 35 be apparent to those skilled in the art to which this invention is directed, I attain by means of the product and the manner of making the same described in the specification 40 and particularly pointed out in the appended claims.

Broadly, my new product consists of a chromium iron alloy base to which a dense, hard coating of tin is applied by electrodeposition. The alloys to which this invention 45 broadly relates are those in which the chromium content is around 12% and the carbon content is not over 14%, but a chromium content of between 9% and 16% is considered 50 around 12%. The carbon content can be any-

thing below 1%. A low carbon content is desirable and necessary when the product is to be subjected to deep stamping operations. 12% carbon has been found satisfactory in many cases, but an even lower carbon 55 content is often desirable.

The chromium iron alloy base may be produced by any desired method, but I prefer to produce the same in an electric furnace of the arc type and to have the alloy as 60 free as possible from oxides and occluded gases.

After the alloy is worked up into sheets, plates or other forms and after it has been treated to remove the scale, and is ground 65 or sand blasted and in some cases polished, it is electroplated with tin.

Before plating, however, it is imperative that the surface to be plated be rendered passive as no satisfactory deposit of tin or 70 other sanitary metal can be obtained unless this is done. In order to render these surfaces passive, I immerse the article to be plated in a solution (preferably warm) of 75 nitric acid which I find can range from a 2% solution to a concentrated solution. I find that a concentrated solution is preferable and that it is only necessary to immerse the articles for a few minutes.

In some way, not known to me, the articles 80 become what I term passive and I find that while the surfaces of the articles remain smooth and polished, if polished before immersion the plating metal will adhere tenaciously which is not the case unless the surface is rendered passive.

I find that it is necessary to use an electroplating process which will not produce a rough, spongy or tree forming deposit and I prefer, therefore, to use a solution of 90 potassium fluoride and tin, as set forth in United States Letters Patent No. 1,423,686, issued to me on July 25, 1922, and as set forth in said patent, I prefer to use from 1 to 2 volts and to have from 10% to 20% of anode 95 surface in proportion to cathode surface since I have found that with these proportions, the solution with a slight acid reaction, is practically self sustaining. In preparing the plating solution, I dissolve, as set forth in 100

said Patent No. 1,423,686, one pound of caustic potash (KOH) in about two quarts of water. To this, I add partly diluted hydrofluoric acid (HF) until acid reaction is obtained, then add sufficient water to make from one to ten gallons in all. In this solution of potassium fluoride having a slight excess of hydrofluoric acid, I suspend metallic tin as an anode or positive bus bar and on the negative bus bar I connect metal strips surrounded by porous cups and with the aid of the electric current I dissolve the metallic tin until the solution has absorbed approximately one ounce of tin per gallon of fluid. I then remove the porous cups and metal strips and suspend the chromium iron alloy articles to be plated. Instead of using the electric current in connection with porous cups for dissolving and saturating a new solution, I may add any soluble tin salt for instance, chloride of tin to the solution.

If it is necessary to have a high lustre or polish on the finished articles, the articles, before being surfaced with tin must be ground and polished in the same manner that articles are prepared today for nickel plating. If only a semi-white lustre or mat finish is required, the articles before being surfaced with tin should be ground or sand blasted and it is advisable after the articles have been surfaced, to scratch brush the same. This treatment of scratch brushing produces an even metallic lustre and if a higher lustre is desired, this can be produced by tumbling the articles in what is commonly known as a ball burnisher.

In order to make the tin coat or surface dense and non-porous and in order to cause the tin to alloy with the base metal or alloy, it is necessary to heat treat the articles after the tin has been deposited and before the articles are finally finished. This can be done in various ways. One way is to place the articles in a furnace and raise the same to a temperature above the melting point of tin for a short time. I have found that by raising the coated articles for a short time to a temperature above the melting point of tin, the tin shrinks and changes its structure and I believe alloys with the base metal or alloy therebeneath. The shrinkage of the tin under this heat treatment is visible to the naked eye.

The time required for this heat treatment depends upon the degree of heat and the weight of the article to be treated. A light gauge sheet which has been tinned, can be heat treated by subjecting it to a temperature of from 1000° to 1500° F. for from one to three minutes.

The tinned articles may also be heat treated by immersing them in a neutral chemical compound having a melting point higher than that of tin, as disclosed in United States Patent No. 1,415,198 issued to me on May 9, 1922.

This chemical compound may be ordinary

commercial saltpetre which is melted in an iron pot by means of a gas flame and in this molten saltpetre I suspend the tinned articles for a few seconds. This produces a bright finish and hardens the tin. If sheets are to be manufactured in large quantities they may be satisfactorily heat treated by passing them between smooth metal rollers raised to a temperature above the melting point of tin.

Having thus described my invention, what I claim is:—

1. The method which consists in subjecting the surfaces of an article made from an iron chromium alloy to the action of a solution of nitric acid in electrodepositing tin on the surfaces so treated and then in hardening the deposited tin. 70

2. The method which consists in rendering the surfaces of an iron chromium alloy article passive, in plating the surface with tin and then in hardening the plating metal. 80

3. The method which consists in passivifying the surface of an iron chromium alloy article, in electrodepositing a sanitary metal on the passivified surface and then in hardening the deposited metal. 90

4. The method which consists in passivifying the surface of an iron chromium alloy article, in depositing a sanitary metal on such passivified surface and then in raising the temperature of the article above the melting point of the sanitary metal. 95

5. The method for producing a non-porous adherent deposit of tin on the surface of an iron chromium alloy, which consists in passivifying the surface of such an alloy, in electro-depositing tin on the passivified surface and then in heating said plated alloy in a furnace having a temperature higher than the melting point of tin. 100

6. The method of producing a non-porous adherent deposit of tin on chromium iron alloys which consists in passivifying said alloys in a 2% solution of nitric acid, in electro-depositing a thin layer of tin on said alloy and in hardening said layer of tin by heating to a temperature above the melting point of tin. 105

7. The method of producing a non-porous adherent deposit of tin on chromium iron alloys which consists in passivifying said alloy in a solution ranging from 2% to concentrated nitric acid, in electro-depositing a thin layer of tin on said passivified alloy and in heat treating said layer of tin. 115

8. The method of producing a non-porous adherent deposit of tin on chromium alloys which consists in passivifying said alloys, in electro-depositing a thin layer of tin on said alloy and then in hardening said plated articles by subjecting to a temperature of from 1,000 to 1,500° F. for at least one minute. 120

9. The method of producing a non-porous adherent deposit of tin on chromium alloys which consists in passivifying said alloys, in 130

electro-depositing a thin layer of tin on said alloy and then in hardening said plated articles by subjecting to a temperature of from 1,000 to 1,500° F. for about three minutes.

5 10. The method of shrinking and hardening electrolytic tin without the aid of fluxes which consists in depositing a thin layer of tin on a passivified base metal and in heating the plated metal in a furnace having a temperature higher than the melting point of tin; said layer of tin being of such thinness that on melting the tin will remain in suspension on the base metal.

10 15. The method of hardening and shrinking electrolytic tin without the aid of fluxes which consists in heat treating the plated metal in a furnace having a temperature above the melting point of tin and in holding the plated metal at that temperature for about 20 three minutes; said electrolytic tin being of such thinness that the tin will not flow on being melted.

In testimony whereof, I have hereunto subscribed my name this 13th day of May, 1926.

25 LOUIS SCHULTE.

30

35

40

45

50

55

60

65